

# UNITED STATES PATENT OFFICE.

JUAN ANIBAL DOMINGUEZ, OF BUENOS AIRES, ARGENTINA.

## DYEING PROCESS.

Specification of Letters Patent.

Patented June 9, 1914.

1,099,240.

No Drawing.

Application filed April 27, 1912. Serial No. 693,724.

To all whom it may concern:

Be it known that I, JUAN ANIBAL DOMINGUEZ, a citizen of Argentina, residing at Buenos Aires, Argentina, have invented a new and useful Dyeing Process, of which the following is a specification.

This invention relates to a method for utilizing the exudations of certain plants as a fixing means for dyes.

10 One object of the invention is to provide a method by means of which the kinos of the white and black algarroba (*Prosopis alba* and *Prosopis nigra*) and the extracts of said kinos may be used for fixing artificial coloring matter to textile fabrics.

15 Other objects will be more clearly understood by reference to the following specification and appended claims.

In a prior application for U. S. Letters 20 Patent, filed October 9, 1911, Serial No. 653,737, I have pointed out that the exudations of the white and black algarroba (*Prosopis alba* and *Prosopis nigra*) have the same tannic and astringent qualities as the exudations usually designated by catechu, kinos or gambier respectively. The extracts of the kino of the algarroba contain about 30% of tannic acid and 38% of catechin. They, therefore, are not only adapted to form the bases for coloring matter and to produce various tints by adding chemical ingredients thereto, but they are also adapted for the purpose of fixing dyes primarily applied to various objects. These dyes may be well known artificial coloring bases, like fuchsin, 35 malachite green or the like.

The exudation forms an insoluble compound with alumina or with metal oxids, and these compounds also serve as fixing means 40 for coloring matters of acid qualities, like alizarin, etc. It will be seen, therefore, that the extracts of the algarroba are not only of substantial value as coloring matter, but also as a fixing means for other coloring matters.

45 The reactions which take place are based on the combination of the coloring matter like fuchsin with the tannic acid and the catechin of the algarroba extracts. The result is, therefore, a colored pigment. In 50 these re-actions also a combination takes place between the coloring basis and an oxid

which is precipitated in the textile and which combines with tannic acid and catechin of the algarroba.

The great value of this discovery for industrial purposes rests in this—that textiles obtain thereby a maximum of color value with a minimum of applied coloring matter after they have been treated in a solution of the kinos of the algarroba. It has also been found that by the application of this method the weight of the textile material is greatly increased. This increase in weight also takes place when the textile (especially silk) is treated with catechu, and is immersed afterward in a solution of iron and zinc salts. The increase by weight of this treatment amounts to 19.5 to 18.71%. If, however, the same material is treated in a solution of kinos of the algarroba and is subjected to the treatment in a solution of iron and zinc salts afterward the increase in weight will amount to from 24 to 24.31%.

In the following various examples are given for utilizing the extracts of the algarroba (*Prosopis alba* and *Prosopis nigra*) as a fixing means for dye stuffs. These examples apply to the treatment of cotton fibers, although they may be used in connection with other textile material when suitable alterations of the method are applied.

For fixing malachite green in cotton the textile is immersed in a bath containing a 12% solution of the kino of the algarroba. The textile is then dried by wringing out and transferred to a bath containing pyrolignite of iron at 3° Baumé. The material is washed and dyed in malachite green, the solution being in the meanwhile slowly heated to the boiling point. After having been dyed the material is washed in a weak solution of soap and water.

For fixing that coloring matter in cotton which comes on the market under the name of "Femilene gray" the material is placed into a bath containing a 10% solution of the kino of the algarroba and is then transferred after having been dried by wringing out, to a 3% bath of tartar emetic or acetate of aluminium. It is again dried, washed and finally the dye is applied in a solution at a temperature of 50°.

I claim:

1. A method of dyeing material which consists in treating the material to be dyed in extracts of algarroba trees (*Prosopis alba* 5 and *Prosopis nigra*), and then applying the dye material in form of bases or acids.
2. A method of fixing dye stuffs in textile materials which consists in immersing the material to be treated in a bath containing

an extract of the algarroba (*Prosopis alba* 10 or *Prosopis nigra*) washing the material and then applying the coloring solution thereto.

In testimony whereof I affix my signature in presence of two witnesses.

JUAN ANIBAL DOMINGUEZ.

Witnesses:

JOSÉ A. GINTIÁN,  
ALBERT G. EBERT.

Copies of this patent may be obtained for five cents each, by addressing the "Commissioner of Patents,  
Washington, D. C."